

## UNITED STATES PATENT OFFICE

2,346,609

## STORING AND SHIPPING HYDROGEN PEROXIDE

Walter S. Riggs, Haddon Heights, N. J., and Rudolf Lehmann, Hollywood, Pa., assignors to The Pennsylvania Salt Manufacturing Company, Philadelphia, Pa., a corporation of Pennsylvania

No Drawing. Application March 17, 1943,  
Serial No. 479,508

4 Claims. (Cl. 148—6)

This invention relates to the passivation of aluminum against attack by hydrogen peroxide.

An object of the invention is to provide a method of treating aluminum, for example, in the form of containers, so that it will withstand attack by hydrogen peroxide.

Another object of this invention is to provide a container of hydrogen peroxide, wherein at least the interior surface of the container is made of aluminum, which may be stored and shipped without incurring any substantial loss of hydrogen peroxide through its interaction with the container.

According to this invention aluminum is treated with a solution of sodium hydrosulfite ( $\text{Na}_2\text{S}_2\text{O}_4$ ) to render it resistant to attack by hydrogen peroxide.

The treatment is preferably applied to the depassivated metal although it may be applied to aluminum containers in which hydrogen peroxide has been shipped previously and which may or may not have been previously passivated.

The essential conditions of the treatment are time, temperature, and concentration of the solution employed.

The time of treatment can be varied. Treatment periods of from about  $\frac{1}{2}$  hour to about forty-eight hours have been employed. Obviously the invention is not limited to any specific time range except that generally speaking longer treatment times are preferred since these result in more durable effects. In general, with higher temperatures, shorter treatment times can be employed.

The temperature of the treatment can be varied. Treatment temperatures of from about 15° C. to about 100° C. have been employed and, in general, a temperature in the range of 35° C. to 100° C. can be employed with good results. As stated, time and temperature are dependent and compensating variables.

The concentration of the treating solution can likewise be varied. Concentrations within the range of from about 1% to about 25% (saturation) can be employed and, in general a concentration in the range of from about 5% to about 20% will be employed.

For example, good results have been obtained by applying a 17% aqueous solution of sodium hydrosulfite to the aluminum at a temperature of about 37° C. for 6 hours. Effective results

have been obtained with a 5% sodium hydrosulfite solution applied to the aluminum at a temperature of about 95° C. for about 1 hour. Other conditions of treatment can be employed and it is to be understood that wide variation of the treating conditions is possible within the scope of the claims. It is obvious that the extent of metal surface treated with a given solution will be limited by the rate at which the sodium hydrosulfite becomes converted or otherwise spent in the solution. Since sodium hydrosulfite is easily oxidized by air, it is advisable to prevent its contact with air during the treatment.

It is preferable, when treating aluminum containers which are to be passivated, to pretreat by boiling them under reflux with a dilute sulfuric acid solution and then rinsing with water.

It will be obvious that the specific treatment selected will depend upon the state of the metal prior to its treatment.

It will also be understood that various conditions will give various degrees of passivation and that those skilled in the art will be able to determine preferred treatments in each case.

We claim:

1. The process of passivating aluminum to enable it to resist attack by hydrogen peroxide which comprises treating it with an aqueous solution of sodium hydrosulfite.

2. The process of claim 1 wherein the solution of sodium hydrosulfite has a concentration in the range of 1% to 25%, the time of treatment is in the range of  $\frac{1}{2}$  hour to 48 hours, and the temperature of treatment is in the range of 15° C. to 100°.

3. The process of claim 1 wherein the solution of sodium hydrosulfite has a concentration in the range of 5% to 20%, the time of treatment is in the range of  $\frac{1}{2}$  hour to 24 hours, and the temperature is in the range of 35° C. to 100° C.

4. The method of passivating a hydrogen peroxide container having an interior surface of aluminum which consists in treating said surface with a 17% aqueous solution of sodium hydrosulfite at a temperature of about 37° C. for about 6 hours.